

Apr. 3, 1923.

1,450,734

E. ROTH

HEAT TREATMENT METHOD OF RENDERING METALS DUCTILE

Filed Jan. 19, 1921



Inventor  
22 Emery Roth,

Chamberlinrendenid  
By A. H. B.

## UNITED STATES PATENT OFFICE.

EMERY ROTH, OF CHICAGO, ILLINOIS.

## HEAT-TREATMENT METHOD OF RENDERING METALS DUCTILE.

Application filed January 19, 1921. Serial No. 438,331.

*To all whom it may concern:*

Be it known that I, EMERY ROTH, a citizen of Hungary, residing at Chicago, county of Cook, State of Illinois, have invented a certain new and useful Improvement 5 in Heat-Treatment Methods of Rendering Metals Ductile, and declare the following to be a full, clear, and exact description of the same, such as will enable others skilled in the art to which it pertains to 10 make and use the same, reference being had to the accompanying drawings, which form a part of this specification.

The present invention relates more particularly to those refractory metals, metal mixtures, and alloys, with or without non-metallic additions, of which tungsten is an example, which can be formed into considerable masses only from an agglomeration 15 of the materials themselves or their compounds in powdered or granular form; the individual particles or grains being united under suitable pressure, with or without the application of binders, into ingots or rods. 20 The object of the present invention is to produce pure refractory metals, mixtures and alloys of the same, with or without non-metallic additions, in the form of comparatively large masses which will be capable of 25 being worked mechanically in a cold state, with possible occasional annealing, in the same manner as the ordinary so-called ductile metals and without requiring mechanical working such as rolling, swaging, drawing, 30 ing., etc., in order to secure ductility.

It is known that if a metal is heated gradually from a minimum temperature, at which no permanent structural change takes place, to a critical temperature, at which 40 the crystalline structure of the metal is permanently changed, or above such critical temperature and close to the melting point of the metal, and then again gradually cooling the metal, the crystallization and the 45 crystal growth can be directed at will. In this way it is possible to obtain a single crystal or a multitude of elongated crystals over a considerable portion or the entire length of a heat treated rod or wire. 50 The present invention is based on this principle.

The various features of novelty whereby my invention is characterized will herein-after be pointed out with particularity in 55 the claims; but, for a full understanding of my invention and of its objects and ad-

vantages, reference may be had to the following detailed description taken in connection with the accompanying drawing, which is a vertical axial section through an 60 apparatus by means of which my invention may be carried out.

In carrying out my invention, I start with a rod or long ingot of the material to be treated. The most important of such materials is tungsten and, for the sake of brevity, I shall confine the detailed description to the process of making ductile tungsten rods and ingots. This rod is formed in any known way of making rods of non-ductile 70 tungsten. This rod is slowly passed through a comparatively short hot zone at a speed less than the speed of crystallization. In the case of tungsten this hot zone should have a temperature of about three thousand 75 degrees centigrade and the speed of travel of the rod through the zone should be about five meters per hour. The rod, which may initially be cool, is thus progressively heated from one end toward the other, the portions 80 which have passed through the heating zone cooling gradually as other parts approach the heating zone. After the rod has been given the treatment just described, it is subjected to a final heat treatment by 85 passing through the same an electric current heavy enough to heat the ingot to a high temperature which, in the case of tungsten, should be about 3350 degrees centigrade. Both heat treatments should be effected in 90 the presence of inert gases or in a vacuum. Referring to the drawing, 1 represents the tungsten rod, the same being held at its upper end in suitable water-cooled jaws, 2, and dipping at its lower end into a mercury well, 3, surrounded by a cooling chamber, 4. Just above the mouth of the mercury well is an annular refractory member 5 whose outer and inner surfaces are both in the form of frustums of cones, the large end 100 of the chamber within the refractory member being directed toward the mouth of the well. The refractory member is preferably made of tungsten, and may conveniently be supported on tungsten posts, 6, rising from 105 the cover, 7, of the cooling chamber for the well. The member 5 forms one of two electrodes between which an arc is adapted to be formed, the other member being an electrode, 8, of carbon or refractory metal 110 mounted at one end of a lever, 9, which is pivotally supported intermediate its ends as

at 10 and is connected at its other end to a rod, 11; the rod, 11, being adapted to extend to a suitable current regulator, not shown, whereby a constant current may be obtained. The mercury well lies below a table, 12, and opens upwardly through the top of the same, the regulating rod, 11, passing down through the table at one side of the wall. Above the table, and surrounding the rod and the water-cooled jaws is a bell, 13, namely a receptacle open at the bottom. This bell is surrounded by a cooling chamber, 14, and its lower edge dips into a suitable mercury trough, 15, resting on the table; the mercury serving to form a gas seal between the table and the bell and at the same time permitting the bell to be raised at will. The bell with its surrounding cooling chamber is held against lateral displacement and guided in its vertical movements by suitable vertical guide rods, 16, projecting upwardly from the table. The water-cooled jaw, 2, is supported on the lower end of a tubular member, 17, which passes out through the top of the bell through a suitable stuffing box, 18. The member 17 serves not only as a support for the work but also as a conduit to permit the introduction of an inert gas under pressure. The table is provided with a small opening, 19, extending through the same within the space enclosed by the bell, so that the inert gas may pass slowly out of the bottom of the chamber.

In starting the heat treatment, the tube, 17, is lowered so that substantially the entire rod or ingot is submerged in the mercury. After the current has been on long enough to raise the temperature of the refractory member 5 to the desired point the tube 17 is slowly lifted so that one portion of the rod after the other is raised out of the mercury, brought into the heating zone, and then passes beyond the heating zone so as gradually to cool.

The final heat treatment may be done in the treating or sintering bottles such as are now used in the manufacture of tungsten, but it can also be done in the apparatus which I have illustrated, the current being passed directly through the rod and being kept as uniform as possible because it has been found desirable to maintain uniform thermal conditions throughout this final heat treatment. Good results can be obtained by continuing this final heat treatment for about the same length of time that it has heretofore been the custom to keep the work in the sintering bottles after it has gone through the various stages of mechanical workings and heat treatments heretofore deemed essential to the production of ductile tungsten, but I prefer to carry on this final heat treatment for considerably longer time than heretofore.

After the final heat treatment the rod or ingot will be found to be so ductile that it may be worked in a cold state in the same way as the so-called ductile metals, with only the occasional annealing that it is usually necessary to give to ductile metals in order to produce certain kinds of products which can only be produced through much working of the metal.

In using the apparatus which I have heretofore described, it may happen that the annulus is not of uniform temperature throughout its entire annular length and, in order to avoid inequalities in the heating of the rod, I have provided means whereby the annulus may be rotated as the rod is lifted. This may conveniently be accomplished by making the mercury well and its cooling chamber rotatable; suitable gearing, 21, being provided for this purpose, and the mercury well and its cooling chamber being supported at the lower end by a suitable step bearing 22. A suitable stuffing box, 23, is provided at the points where the well and its cooling chamber pass through the table, this stuffing box serving to prevent the escape of the inert gas within the well.

I claim:

1. The method of producing a comparatively large body of ductile tungsten which consists in forming a rod or long ingot of non-ductile tungsten, passing it slowly through a short heating zone having a temperature equal to or above the critical temperature at which the crystalline structure of the tungsten permanently changes and keeping that part of the rod or ingot which has not reached the heating zone cool.

2. The method of producing a comparatively large body of ductile tungsten which consists in forming a rod or long ingot of non-ductile tungsten, passing it slowly through a short heating zone having a temperature of about 3000 degrees C. and, during this operation, keeping that part of the rod or ingot which has not reached the heating zone cool and permitting that part which has passed beyond the heating zone gradually to cool.

3. The method of producing a comparatively large body of ductile tungsten which consists in forming a rod or long ingot of non-ductile tungsten, passing it slowly through a short heating zone having a temperature of about 3000 degrees C. and, during this operation, keeping that part of the rod or ingot which has not reached the heating zone cool and permitting that part which has passed beyond the heating zone gradually to cool, and afterwards passing through the rod or ingot an electric current sufficiently great to heat it to a temperature considerably higher than the aforesaid temperature.

4. The method of producing a compara-

tively large body of ductile tungsten which consists in forming a rod or long ingot of non-ductile tungsten, placing the same in a mercury well, and raising it slowly out of the well and passing it through a short heating zone located above the well and having a temperature of approximately 3000 degrees C.

5. The method of producing a comparatively large body of ductile tungsten which consists in forming a rod or long ingot of non-ductile tungsten, passing the same slowly through an annulus heated to a temperature equal to or above the critical tem-

10 15 20

perature at which the crystalline structure of the tungsten permanently changes and, during this operation, keeping that part of the ingot which has not yet reached the annulus cool and permitting that part which has passed through the annulus gradually to cool.

6. The method of producing a comparatively large body of ductile tungsten which consists in forming a rod or long ingot of non-ductile tungsten, passing the same slowly to an annulus having an internal cross sectional area decreasing gradually in size in the direction of travel of the rod or ingot and heated to a temperature of about 3000 25 30

degrees C. and, during this operation, keeping that part of the ingot which has not yet reached the annulus cool and permitting that part which has passed through the annulus gradually to cool.

7. The method of forming a comparatively large body of ductile metal from an agglomeration of small pieces of the metal or its compounds, which consists in pressing a mass of the material into a rod or long ingot, passing the rod or ingot slowly through a short heating zone having a temperature at or above the critical temperature at which the crystalline structure of the metal changes permanently and, during this operation, keeping cool that part of the rod or ingot which has not reached the heating zone and permitting that part which has passed said zone gradually to cool.

8. The method of forming a comparatively large body of ductile metal from an agglomeration of small pieces of the metal or its compounds, which consists in pressing a mass of the material into a rod or long ingot, passing the rod or ingot slowly through a short heating zone having a temperature at or above the critical temperature at which the crystalline structure of the metal changes permanently and, during this operation, keeping cool that part of the rod or ingot which has not reached the heating zone and permitting that part which has passed said zone gradually to cool; and afterwards heating the entire rod or ingot to a temperature considerably higher than that of the heating zone.

In testimony whereof, I sign this specification.

EMERY ROTH.